

Patented Jan. 9, 1945

2,366,714

# UNITED STATES PATENT OFFICE

2,366,714

## ELECTROLYTE FOR AND METHOD OF ANODICALLY POLISHING COPPER

Charles L. Faust, Columbus, Ohio, assignor to Battelle Memorial Institute, Columbus, Ohio, a corporation of Ohio

No Drawing. Application April 24, 1942,  
Serial No. 440,337

5 Claims. (CL 204—140)

This invention relates to a phosphoric acid containing electrolyte for anodically polishing copper. The invention further pertains to methods of electropolishing copper in such an electrolyte.

A bath heretofore preferred for the anodic polishing of copper consists of 75% to 85% orthophosphoric acid saturated with chromic acid. Depending on the temperature at which the chromic acid is dissolved in the phosphoric acid, the composition of this bath will range from 69% orthophosphoric acid and 7% chromic acid to 81% orthophosphoric acid and 5% chromic acid. Minimum initial current densities of 250 to 300 or even more amperes per square foot at tank voltages of 8 to 10 volts are required, and these minima are increased progressively as the bath is used. The viscosity of the phosphoric acid-chromic acid bath is also somewhat high, causing excessive drag out loss of electrolyte.

Orthophosphoric acid can be used alone for electro-polishing copper, but only at the impractically low temperature of 70° F. The addition of hexavalent chromium in the form of chromic acid thus serves to make possible electropolishing of copper in phosphoric acid at practically feasible temperatures. But the progressive rise in current density and tank voltage characteristic of chromic acid containing phosphoric acid baths is thought to be due to this chromic acid addition, being caused, more particularly, by continuous reduction of hexavalent chromium to trivalent chromium and by continuous accumulation in the bath of anodically dissolved copper.

I have now found that the addition of trivalent aluminum and, optionally, trivalent chromium, to phosphoric acid containing copper polishing baths renders the baths less viscous and makes possible electropolishing at lower current densities, tank voltages and temperatures. Further, the dissolved copper is plated out cathodically in recoverable form from such baths, so that continuous operation is greatly facilitated and maintenance can be effected simply by replacing dragged-out electrolyte and decomposed water.

It is, therefore, an important object of the present invention to provide an electrolyte for the anodic polishing of copper containing phosphoric acid and trivalent aluminum together with trivalent chromium as an optional ingredient.

Another important object of this invention is to provide methods for anodically polishing copper in phosphoric acid at low current densities and tank voltages operative at commercially desirable temperatures.

A further important object of the invention is to provide methods for continuously electropolishing copper in an electrolyte from which anodically dissolved copper is plated out cathodically in easily recoverable form.

Still another object of the invention is to pro-

vide an electrolyte for the anodic polishing of copper characterized by substantially constant current density and tank voltage in continuous use and maintainable by simple additions to replace decomposed water and dragged out electrolyte.

Other and further objects and features of the present invention will become apparent from the following description and the appended claims.

10 In general, the baths of the present invention contain preferably about 75 to 84% (by weight) of 100% orthophosphoric acid, about from 0.25 to 2.0% or, preferably, 0.3 to 1.5% trivalent aluminum, from 0 to 2% trivalent chromium, and, 15 after having been used, about from 0.3 to 0.5 up to 1% copper, the balance being largely water. Such baths produce, with little or no agitation, a brilliant, mirror-like finish on copper at temperatures of from 100° to 125° or 130° F. at current densities of from 50 to 200 or, preferably, 100 to 150 amperes per square foot and tank voltages sometimes as low as 4 or 5 volts. The usual copper content of such baths is about 0.4 to 0.5%. Additional copper dissolved anodically 20 is plated out on the cathodes where the copper may be recovered as a fine powder consisting of 98% or purer copper. Hence, the baths can be used continuously, with very simple chemical control and maintenance. The only replacements required are those compensating for loss of decomposed water and for a limited amount of loss due to dragging out of the not very viscous electrolyte. The new baths are further less corrosive than chromic acid-containing phosphoric acid baths, and can be handled and used in lead lined equipment. The treating times are the same, or shorter, than those used in chromic acid containing phosphoric acid baths, and, apart from the features mentioned, the baths of the present invention are used as are chromic acid containing phosphoric acid baths.

Specific examples of baths according to the present invention have the following compositions:

|    |                                | Bath No. 1         | Bath No. 2         |
|----|--------------------------------|--------------------|--------------------|
|    |                                | Per cent by weight | Per cent by weight |
| 60 | H <sub>3</sub> PO <sub>4</sub> | 75                 | 82                 |
|    | Cr <sup>3+</sup>               | <0.8               | 0.5                |
|    | Al <sup>3+</sup>               | 0.3-0.6            | 0.4                |
|    | Cu                             | 0.3-0.5            | 0.4                |
|    | Water                          | Balance            | Balance            |

55 Bath No. 1 may be prepared by adding a trivalent chromium salt to 75% orthophosphoric acid, the required amount of aluminum metal having been dissolved in the phosphoric acid by heating. For instance, chromic chloride may be dissolved in the phosphoric acid, the resulting

solution being heated until all the hydrochloric acid has been driven off, as evidenced by the absence of smoke formation on blowing ammonia fumes over the bath. The latter will then have been evaporated off to about two-thirds of its original volume. Before the bath is used, water is added to restore the bath to its original volume.

Bath No. 1 may also be prepared by starting with a bath containing 84% orthophosphoric acid, 1% chromic acid and 0.5% metallic aluminum dissolved in the phosphoric acid, this bath being electrolyzed and water being added to the bath until all the hexavalent chromium has been reduced to trivalent chromium.

Bath No. 2 may be prepared similarly to bath No. 1.

Copper is electropolished in bath No. 1, with very little or no agitation, to a brilliant, mirror-like finish at 100 to 200 amperes per square foot at a temperature of from 110° to 125° F. Bath No. 2 electropolishes copper well at a current density of 150 amperes per square foot at a temperature of 120° F. The operative temperature ranges at various current densities for bath No. 2 after aging are set forth in the following table:

Table I

| Current density in amperes per square foot | Minimum practical temperature for good polishing | Maximum temperature for good polishing | 35 |
|--------------------------------------------|--------------------------------------------------|----------------------------------------|----|
|                                            | °F.                                              | °F.                                    |    |
| 50                                         | 100                                              | 110                                    |    |
| 100                                        | 105                                              | 130                                    |    |
| 150                                        | 110                                              | 150                                    |    |
| 200                                        | 110                                              |                                        |    |
| 250                                        | 110                                              |                                        |    |

Temperatures lower than the indicated minima may be employed but then provisions must be made for cooling the baths. At current densities of at least 200 amperes per square foot, temperatures of 170° F. or higher may be employed with good results.

Although in both bath No. 1 and in bath No. 2 the electropolishing time depends on the nature of the copper and the starting surface, it has been noted that bath No. 2 requires a slightly longer time than bath No. 1, which has greater anode efficiency.

The relative effect of temperature on cell voltage and current efficiency at various current densities in bath No. 2 after aging is shown by Table II.

Table II

| Current density in amps. per sq. ft. | 110° F.             |                 | 120° F.             |                        | 135° F.         |                     | 70                     |                 |
|--------------------------------------|---------------------|-----------------|---------------------|------------------------|-----------------|---------------------|------------------------|-----------------|
|                                      | Cell volt. in volts | Char. of polish | Cell volt. in volts | curr. eff. in per cent | Char. of polish | Cell volt. in volts | curr. eff. in per cent | Char. of polish |
| 50                                   | 3.2                 | Good            | 3.0                 | 50                     | Def.            | 3.4                 | 58                     | Defec.          |
| 100                                  | 4.0                 | do              | 3.8                 | 35                     | Good            | 3.4                 | 43                     | do              |
| 150                                  | 4.6                 | do              | 4.4                 | 35                     | do              | 3.8                 | 43                     | do              |
| 200                                  | 5.1                 | do              | 4.8                 | 35                     | do              | 4.1                 | 42                     | Good            |
| 250                                  | —                   | 4.9             | 38                  | do                     | —               | 4.4                 | 42                     | do              |

If the water concentration is over 23 to 25% in the type of bath exemplified by baths Nos. 1 and 2, good electropolishing is not secured at a current density below 150 amperes per square foot, at temperatures above 110° F., or at a metal concentration (including the total concentration

of divalent copper, trivalent chromium and trivalent aluminum) of less than 2.5%. The influence of dilution on cell voltage and current efficiency when electropolishing at 120° F. and a current density of 150 amperes per square foot is indicated in the following table:

Table III

| Specific gravity of bath at 25° C. | Concen- tration of $H_3PO_4$ in percent | 0.5% $Al^{3+}$ —1.2% $Cr^{3+}$ |                                         | 0.5% $Al^{3+}$ —0.5% $Cr^{3+}$ |                                         |
|------------------------------------|-----------------------------------------|--------------------------------|-----------------------------------------|--------------------------------|-----------------------------------------|
|                                    |                                         | Cell volt- age in volts        | Anode cur- rent effi- ciency in percent | Cell volt- age in volts        | Anode cur- rent effi- ciency in percent |
| 1.74                               | 84                                      | 6                              | 35                                      | 5.8                            | 39                                      |
| 1.72                               | —                                       | 5.6                            | 35                                      | 5.3                            | 39                                      |
| 1.70                               | —                                       | 5.4                            | 35                                      | 5                              | 39                                      |
| 1.68                               | —                                       | 5.3                            | 36                                      | 4.9                            | 41                                      |
| 1.66                               | —                                       | 5.2                            | 38                                      | 4.8                            | 43                                      |
| 1.64                               | —                                       | 5.1                            | 39                                      | 4.7                            | 44                                      |
| 1.62                               | 74                                      | 5                              | 40                                      | 4.6                            | 44                                      |

The lower operative current densities at 120° F. are indicated in Table IV, which also serves to show the necessity for including trivalent aluminum with the bath to secure satisfactory electro-polishing.

Table IV

| Current density in amps. per sq. ft. | 76% $H_3PO_4$ , 0.5% Al |                                       |                 | 84% $H_3PO_4$ , 0.5% Al |                                       |                 |
|--------------------------------------|-------------------------|---------------------------------------|-----------------|-------------------------|---------------------------------------|-----------------|
|                                      | Cell volt- age in volts | Anode current effi- ciency in percent | Char. of polish | Cell volt- age in volts | Anode current effi- ciency in percent | Char. of polish |
| 50                                   | —                       | —                                     | —               | 3.5                     | 39                                    | Defect.         |
| 75                                   | 3.5                     | Good                                  | do              | 4.1                     | 34                                    | Good.           |
| 100                                  | 3.9                     | 45                                    | do              | 4.6                     | 33                                    | Do.             |
| 125                                  | 4.4                     | 42                                    | do              | 5.1                     | 33                                    | Do.             |
| 150                                  | 4.8                     | 40                                    | do              | 5.6                     | 33                                    | Do.             |
| 175                                  | 5.3                     | 40                                    | do              | 6.2                     | 33                                    | Do.             |

  

| 45  | 77% $H_3PO_4$           |                                       |                 | 85% $H_3PO_4$           |                                       |                 |
|-----|-------------------------|---------------------------------------|-----------------|-------------------------|---------------------------------------|-----------------|
|     | Cell volt- age in volts | Anode current effi- ciency in percent | Char. of polish | Cell volt- age in volts | Anode current effi- ciency in percent | Char. of polish |
| 50  | —                       | —                                     | —               | 3.3                     | 44                                    | Defec.          |
| 75  | 3.2                     | —                                     | —               | 3.8                     | 36                                    | Do.             |
| 100 | 3.5                     | 46                                    | Defec.          | 4.3                     | 32                                    | Do.             |
| 125 | 3.9                     | 42                                    | do              | 4.8                     | 29                                    | Do.             |
| 150 | 4.3                     | 38                                    | do              | 5.3                     | 27                                    | Do.             |
| 175 | 4.6                     | 36                                    | do              | 5.8                     | 26                                    | Do.             |

Table V further indicates the critical importance of the aluminum content of the baths according to the present invention. This table further shows that the presence and concentration of chromium are not critical. This table is in-

cluded more specifically as illustrating the effect of the chromium concentration on electropolishing in orthophosphoric acid at 120° F. and a current density of 150 amperes per square foot. The aluminum and the chromium additions were made to a bath containing 85%  $H_3PO_4$ .

Table V

| Trivalent chromium concentration in percent | 0.5% aluminum         |                               |                  | No aluminum           |                               |                  |
|---------------------------------------------|-----------------------|-------------------------------|------------------|-----------------------|-------------------------------|------------------|
|                                             | Cell voltage in volts | Anode current eff. in percent | Nature of polish | Cell voltage in volts | Anode current eff. in percent | Nature of polish |
| 0.....                                      | 5.6                   | 35                            | Good             | 5.1                   | 28                            | Dull satin.      |
| 0.2.....                                    | 5.6                   | 35                            | do               | 5.15                  | 29                            | Do.              |
| 0.4.....                                    | 5.6                   | 35                            | do               | 5.25                  | 30                            | Do.              |
| 0.6.....                                    | 5.6                   | 35                            | do               | 5.3                   | 30                            | Do.              |
| 0.8.....                                    | 5.6                   | 35                            | do               | 5.25                  | 31                            | Do.              |
| 1.0.....                                    | 5.65                  | 35                            | do               | 5.45                  | 32                            | Fair.            |
| 1.2.....                                    | 5.8                   | 34                            | do               | 5.5                   | 33                            | Do.              |

The necessity for a minimum aluminum content is still further shown in Table VI which directly shows the influence of various aluminum concentrations on the nature of the electropolish as well as on the cell voltage and the current efficiency at 120° F. and a current density of 150 amperes per square foot.

Table VI

| Al concentration in percent | 77% H <sub>3</sub> PO <sub>4</sub> |                               |                 | 85% H <sub>3</sub> PO <sub>4</sub> |                               |                 |
|-----------------------------|------------------------------------|-------------------------------|-----------------|------------------------------------|-------------------------------|-----------------|
|                             | Cell voltage in volts              | Anode current eff. in percent | Char. of polish | Cell voltage in volts              | Anode current eff. in percent | Char. of polish |
| 0.....                      | 4.4                                | 38                            | Defect.         | 5.5                                | 26                            | Defect.         |
| 0.25.....                   | 4.6                                | 39                            | Good            | 5.75                               | 32                            | Good.           |
| 0.50.....                   | 4.75                               | 40                            | do              | 5.9                                | 33                            | Do.             |
| 0.75.....                   | 4.9                                | 38                            | do              | 6.1                                | 33                            | Do.             |
| 1.00.....                   | 5.0                                | 38                            | do              | 6.2                                | 33                            | Do.             |
| 1.25.....                   | 5.05                               | 38                            | do              | 6.35                               | 33                            | Do.             |
| 1.50.....                   | 5.1                                | 38                            | do              | 6.5                                | 33                            | Do.             |

The effect at 120° F. and a current density of 150 amperes per square foot of aging on baths according to the present invention and on baths containing phosphoric acid saturated with chromic acid is shown by Table VII, which also indicates the influence of cathode size. The progressive deterioration due to high chromic acid content is evident.

Table VII

| Per cent copper dissolved at anode | Original bath composition 84% H <sub>3</sub> PO <sub>4</sub> , 1% CrO <sub>3</sub> , 0.5% Al |                |                          |                | Original bath composition 81% H <sub>3</sub> PO <sub>4</sub> , 5% CrO <sub>3</sub> |                       |                |                       |               |
|------------------------------------|----------------------------------------------------------------------------------------------|----------------|--------------------------|----------------|------------------------------------------------------------------------------------|-----------------------|----------------|-----------------------|---------------|
|                                    | Cell voltage in volts                                                                        |                | Current eff. in per cent |                | Char. of pol.                                                                      | Cell voltage in volts |                | Cur. eff. in per cent | Char. of pol. |
|                                    | 5/8" cathode                                                                                 | 2 1/4" cathode | 5/8" cathode             | 2 1/4" cathode |                                                                                    | 5/8" cathode          | 2 1/4" cathode |                       |               |
| 0.....                             | 5.7                                                                                          | 4.8            | 34                       | 34             | Good                                                                               | 5.0                   | 42             | Good                  | Good          |
| 2.....                             | 5.7                                                                                          | 4.6            | 34                       | 34             | do                                                                                 | 5.5                   | 41             | do                    | do            |
| 4.....                             | 5.7                                                                                          | 4.4            | 34                       | 34             | do                                                                                 | 5.9                   | 35             | do                    | do            |
| 6.....                             | 5.6                                                                                          | 4.4            | 34                       | 34             | do                                                                                 | 6.3                   | 30             | Def.                  | do            |
| 8.....                             | 5.4                                                                                          | 4.4            | 34                       | 34             | do                                                                                 | 6.4                   | 30             | do                    | do            |
| 10.....                            | 5.3                                                                                          | 4.4            | 34                       | 34             | do                                                                                 | 6.4                   | 30             | do                    | do            |
| 12.....                            | 5.3                                                                                          | 4.4            | 34                       | 34             | do                                                                                 | 6.4                   | 30             | do                    | do            |
| 14.....                            | 5.3                                                                                          | 4.4            | 34                       | 34             | do                                                                                 | 6.4                   | 30             | do                    | do            |

The bath having an original composition including 84% H<sub>3</sub>PO<sub>4</sub>, 1% CrO<sub>3</sub> and 0.5% Al is similar to bath No. 2 discussed on page 4. The amounts of copper indicated as dissolved do not necessarily indicate a corresponding copper content in the baths, since some of the dissolved copper will be plated out. In the case of the aluminum containing baths, copper is plated out when the copper concentration reaches 0.5%. In baths containing chromic acid, the upper solubility limit for copper is from 4% to 6%.

Tables VIII and IX further show the influence of cathode size and of chromium content on aged baths at 120° F.

Table VIII

| Current density in amps. per sq. ft. | 82% H <sub>3</sub> PO <sub>4</sub> , 0.5% Cr, 0.4% Al |                 |                       |                 | 77% H <sub>3</sub> PO <sub>4</sub> -2.4% Cr (from CrO <sub>3</sub> ) 0.2% Al |                 |
|--------------------------------------|-------------------------------------------------------|-----------------|-----------------------|-----------------|------------------------------------------------------------------------------|-----------------|
|                                      | 2 1/4" cathode                                        |                 | 5/8" cathode          |                 | 5/8" cathode                                                                 |                 |
| 10.....                              | Cell voltage in volts                                 | Char. of polish | Cell voltage in volts | Char. of polish | Cell voltage in volts                                                        | Char. of polish |
| 50.....                              | 3.0                                                   | Defec.          | 3.2                   | Defec.          | 3.5                                                                          | Defec.          |
| 100.....                             | 3.8                                                   | Good            | 4.3                   | Good            | 4.8                                                                          | Do.             |
| 150.....                             | 4.4                                                   | do              | 5.2                   | do              | 5.1                                                                          | Do.             |
| 200.....                             | 4.8                                                   | do              | 6.0                   | do              | 7.3                                                                          | Do.             |

Bath No. 2

| Current density in amps. per sq. ft. | 77% H <sub>3</sub> PO <sub>4</sub> , 2.4% Cr <sup>3+</sup> , 0.3% Al <sup>3+</sup> , 0.6% Cu <sup>2+</sup> |                 |                       | 76% H <sub>3</sub> PO <sub>4</sub> , 0.5% Cr <sup>3+</sup> , 0.4% Al <sup>3+</sup> , 0.5% Cu <sup>2+</sup> |                       |                 | 82% H <sub>3</sub> PO <sub>4</sub> , 0.5% Cr <sup>3+</sup> , 0.4% Al <sup>3+</sup> , 0.5% Cu <sup>2+</sup> |                 |                       |        |
|--------------------------------------|------------------------------------------------------------------------------------------------------------|-----------------|-----------------------|------------------------------------------------------------------------------------------------------------|-----------------------|-----------------|------------------------------------------------------------------------------------------------------------|-----------------|-----------------------|--------|
|                                      | Cell voltage in volts                                                                                      | Char. of polish | Cell voltage in volts | Char. of polish                                                                                            | Cell voltage in volts | Char. of polish | Cell voltage in volts                                                                                      | Char. of polish | Cell voltage in volts |        |
| 25.....                              | 3.5                                                                                                        | Defec.          | 3.1                   | Defec.                                                                                                     | 3.2                   | Defec.          | 3.5                                                                                                        | Defec.          | 3.5                   | Defec. |
| 30.....                              | 4.8                                                                                                        | do              | 4                     | Good                                                                                                       | 4.6                   | do              | 4.3                                                                                                        | Good            | 4.3                   | Good   |
| 60.....                              | 6                                                                                                          | do              | 4.6                   | do                                                                                                         | 5.4                   | do              | 5.4                                                                                                        | Do.             | 5.4                   | Do.    |
| 100.....                             | 7.2                                                                                                        | do              | 4.8                   | do                                                                                                         | 6                     | do              | 6                                                                                                          | Do.             | 6                     | Do.    |

Bath No. 1

Bath No. 2

Tables I to IX include data showing that the inclusion of trivalent aluminum with phosphoric acid makes possible continuous electropolishing of copper in the resulting bath, dissolved copper being recovered as electropolishing is continued. The presence of limited amounts of trivalent chromium is not harmful, but does not add to the efficiency of the bath. A larger cathode area lowers cell voltage and raises current efficiency for plating out copper during electropolishing.

40

35

30

25

20

15

10

5

0

5

10

15

20

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

of copper containing from 75 to 84% by weight ortho phosphoric acid, from 0.25 to 2% trivalent aluminum, and from 0.3 to 1% divalent copper, the balance comprising essentially water.

3. The method of electrolytically polishing copper which comprises making the copper the anode in an electrolyte comprising from 75 to 84% by weight ortho phosphoric acid and from 0.25 to 2% trivalent aluminum, the balance comprising essentially water, and at a temperature of at least 100° F. passing current therethrough of sufficient density and for a sufficient period of time to effect a polish on said copper.

4. The method of electrolytically polishing copper which comprises making the copper the anode in an electrolyte containing from 75 to 84% by weight ortho phosphoric acid, from 0.25 to 2% trivalent aluminum, and from 0.3 to 1% divalent copper, the balance comprising essentially water, and at a temperature of at least 100° F. passing current through said electrolyte at a sufficient current density and for a sufficient period of time to effect a polish on said copper.

5. The method of electrolytically polishing cop-

per which comprises making the copper the anode in an electrolyte containing from 75% to 84% by weight orthophosphoric acid, from 0.25% to 2% trivalent aluminum, and from 0.3 to 1% divalent copper, the balance comprising essentially water, and passing a current through said electrolyte at a temperature of from 100° to 170° F. at a current density of from 50 to 250 amperes per square foot, the exact current density depending upon the temperature as indicated by the following table:

| Current density and amperes per square foot | Minimum temperature<br>°F. | Maximum temperature<br>°F. |
|---------------------------------------------|----------------------------|----------------------------|
| 15                                          |                            |                            |
| 50                                          | 100                        | 110                        |
| 100                                         | 105                        | 130                        |
| 150                                         | 110                        | 150                        |
| 200                                         | 110                        | 170                        |
| 250                                         | 110                        | 170                        |

said current being passed through said electrolyte for a sufficient period of time to effect a polish on said copper.

CHARLES L. FAUST.